

1,384,470.

W. H. KEMPTON,  
OIL RING,  
APPLICATION FILED SEPT. 3, 1919.

Patented July 12, 1921.

Fig.1.



Fig. 2.



Fig. 3.



WITNESSES:

*Lead Barrett*  
*O. E. Bee.*

INVENTOR  
*Willard H. Kempton.*  
BY  
*Wesley G. Barr*  
ATTORNEY

# UNITED STATES PATENT OFFICE.

WILLARD H. KEMPTON, OF WILKINSBURG, PENNSYLVANIA, ASSIGNOR TO WESTINGHOUSE ELECTRIC & MANUFACTURING COMPANY, A CORPORATION OF PENNSYLVANIA.

## OIL-RING.

1,384,470.

Specification of Letters Patent. Patented July 12, 1921.

Application filed September 3, 1919. Serial No. 321,495.

*To all whom it may concern:*

Be it known that I, WILLARD H. KEMPTON, a citizen of the United States, and a resident of Wilkinsburg, in the county of 5 Allegheny and State of Pennsylvania, have invented a new and useful Improvement in Oil-Rings, of which the following is a specification.

My invention relates to oil rings and it 10 has, for its primary object, the provision of oil rings formed of a moldable composition reinforced by a fibrous material in such manner as to insure a strong and durable product.

15 It has been customary, heretofore, to employ oil rings formed of various metals, some of which are relatively expensive and also result in heavier devices than are demanded by the functions to be performed.

20 Furthermore, metallic rings are objectionable for the reason that they must be carefully handled before they are disposed in their operative positions because some of them are brittle and are, therefore, easily 25 broken when subjected to shocks, while others, formed of other metals, may become rusted, if exposed to the weather.

One object of my invention resides in the 30 provision of an oil ring which is unaffected by moisture, oils, weak acids, alkalis and relatively wide temperature changes.

Another object of my invention is the 35 construction of oil rings which shall be comparatively light in weight and possess relatively great mechanical strength.

With these and other objects in view, my 40 invention will be more fully described, illustrated in the drawings, in the several views of which corresponding numerals indicate like parts, and then particularly pointed out in the claims.

In the drawings, Figure 1 is a sectional 45 view, parts being broken away, of a bearing end of a motor and an oil ring, constructed in accordance with my invention, disposed in position upon the shaft of the motor; Fig. 2 is a side elevation of an oil ring embodying my invention, and Fig. 3 is a diametral sectional view of the ring 50 shown in Fig. 2.

In practising my invention, I may construct an oil ring by employing a moldable composition comprising a comminuted material mixed with a suitable binder. The

binder and comminuted material may be 55 disposed in a mold, and reinforcing strands of fibrous material may be disposed in the composition and heat and pressure be applied thereto to compact the material and to harden the binder. 60

In Figs. 2 and 3 is shown an oil ring 1 constructed in accordance with my invention. The oil ring may be constructed by employing a comminuted material, such as wood flour, which may be mixed with a 65 phenolic condensation product, in a dry or powdered form. A suitable quantity of such a mixture may be disposed in a mold, and strands 2 of fibrous material, such as cord, may be disposed in the material to act as a 70 reinforcing body. The material may be subjected to heat and pressure to compact it and to first soften the phenolic condensation product and to then harden it.

Although an article formed of a com- 75 minuted material, such as wood flour, mixed with a binder, such as phenolic condensation product, is somewhat brittle in character, the reinforcing strands I employ materially increase the mechanical strength of the 80 resulting product and obviate the danger of the rings being broken when subjected to shocks. The material is relatively inexpensive and insures a product which is light 85 in weight and practically unaffected by chemicals or moisture.

Furthermore, the oil rings, constructed as 90 above described, possess exceptionally durable wearing qualities which may be compared favorably with metals which are relatively expensive and difficult to handle. The wood flour may be the predominant portion of the total quantity of material employed, but the proportions of wood flour and the phenolic condensation product may be varied 95 rather widely. However, I have found that approximately 50% of the total quantity of material should be a binding agent, such as a phenolic condensation product.

Although I have specifically described 100 oil rings which may be constructed in accordance with my invention, it is obvious that minor changes may be made in their construction without departing from the spirit of my invention, and I desire, therefore, that no limitations shall be imposed 105 except such as are indicated in the appended claims.

I claim as my invention:—

1. An oil ring comprising a comminuted material associated with a hardened binder and reinforcing strands of fibrous material disposed therein.
2. An oil ring comprising a comminuted material associated with a hardened phenolic condensation product and reinforcing strands of fibrous material disposed therein.
- 10 3. An oil ring comprising wood flour associated with a hardened binder and reinforcing strands of fibrous material disposed therein.
4. A molded oil ring comprising a comminuted material associated with a hardened binder and reinforcing strands of fibrous material disposed therein.
5. A molded oil ring comprising wood flour associated with a hardened phenolic condensation product and reinforcing wind- 20 ings of cord disposed therein.

In testimony whereof I have hereunto subscribed my name this 25th day of Aug. 1919.

WILLARD H. KEMPTON.